

## UNITED STATES PATENT OFFICE

2,083,143

## EXPLOSIVES

Laud S. Byers, Glendale, Calif., assignor, by  
mesne assignments, to Halifax Explosives Com-  
pany, Los Angeles, Calif., a corporation of Del-  
aware

No Drawing. Application August 20, 1934,  
Serial No. 740,636

7 Claims. (Cl. 52—13)

This invention relates to a method of compounding ingredients for use in explosive compositions and to combinations of specified ingredients in particular proportions whereby an explosive characterized by stability to temperature changes, or protracted exposure to high temperatures, ease and cheapness of manufacture, water resistance, and ability to propagate and detonate with great efficiency is obtained.

Although there are numerous compounds and compositions which may be termed to be explosives because they will detonate when set off with a fulminating cap, very few of such compositions or compounds are adapted for actual commercial manufacture and use. In addition to detonating ability, an explosive must fulfill a number of separate and distinct requirements, among them the following: the explosive should not freeze or become insensitive at low temperatures; it should not bleed or liberate a liquid constituent upon exposure to high temperatures; it should not harden with age; it should maintain a relatively sticky, moldable constituency capable of being rammed into upwardly directed holes without falling out; it should not liberate noxious fumes upon explosion; it should be capable of withstanding percussion, blows and rough handling; upon being ignited in the open, it should not burn with great rapidity or with explosive force; it should not be subject to ignition by a sputtering fuse; upon being detonated in a hole, additional sticks of the explosive separated more than one inch from the original stick, should also detonate instantaneously.

Explosives answering individual requirements have been made heretofore but none of the explosives of the prior art answered all of these requirements. This invention, however, is directed to a combination of specific ingredients in specific proportions which result in an explosive answering all of the above requirements.

Nitrated cellulose varies in nitrogen content and this invention contemplates the use of nitrated cellulose containing 12% or more of nitrogen.

More specifically stated, the invention in part relates to a method whereby more nitrated cellulose, containing more than 12% of nitrogen, may be mixed together into stable solution in a liquid mixture of isomers of dinitrotoluene, a result which has not been attained heretofore. The solution thus obtained is eminently suited for use in various explosives, particularly in explosives containing chlorates and nitrates. The resulting solution increases the efficiency of the final explo-

sive compound whereas suspensions or dispersions of nitrocellulose in such mixture of isomers has a tendency to deaden and reduce the propagating and detonating characteristics of an explosive compound.

A still further object of the present invention is to disclose and provide a complete explosive compound in which a relatively shredded wood is used instead of the customary ground wood flour or wood pulp. Heretofore, the art has believed that in order to produce an efficient explosive it was necessary to grind and combine the ingredients in a very extreme state of fineness so as to obtain a perfectly homogeneous uniform mixture of all of the ingredients. I have found, on the other hand, that when certain of the ingredients, such as the wood, are ground very fine or are used in the form of flour, effects of much lower efficiency are obtained than is the case when the wood is shredded and has an appreciable and definite size. The shredded particles of wood have a tendency to inter-weave with each other, increasing the plastic moldability of the explosive compound, thus holding it in place when packed into upright or vertical drill holes.

It is an object of this invention, therefore, to disclose and provide an explosive of great power, said explosive being characterized by an absence of noxious fumes upon explosion and by its ability to maintain a moldable plastic form upon storage or exposure to varying temperatures.

Another object of the invention is to disclose and provide an explosive composition which is water-resistant and which may be used in wet holes without impairment of its detonating, rendering and disruptive effects.

A further object is to disclose and provide as an ingredient for use in explosive compositions a stable solution of nitrocellulose containing more than 12% of nitrogen in a mixture of isomers of dinitrotoluene.

A still further object of the invention is to disclose and provide a method of dissolving nitrocellulose containing more than 12% of nitrogen in a liquid mixture of isomers of dinitrotoluene.

These and other objects, uses and advantages of the invention will be apparent to those skilled in the art from the following detailed description of the ingredients, their manner of compounding, and the proportions in which they are to be combined.

As stated hereinabove, the highly nitrated cottons are not soluble in solvents whereas cottons of low nitration, such as collodion cotton containing less than 10% of nitrogen is soluble. The

physical properties of a solution of nitrated cotton in a solvent differ greatly from the physical properties of a suspension of nitrated cotton in the same solvent. Highly nitrated cotton, for example, is not soluble in a liquid mixture of isomers of dinitrotoluene but instead results in the formation of a suspension. This suspension is of increased viscosity but has the property of absorbing appreciable quantities of water. As a result, explosive compounds containing such suspension are not water-resistant. It has been discovered that if nitrated cotton, that is nitrocellulose containing more than about 12% of nitrogen, is first dissolved in a volatile solvent, such as ethyl acetate, acetone, amyl acetate, and the like, and the solution thus obtained then incorporated and mixed with the liquid mixture of isomers of dinitrotoluene with which such nitrocellulose-solvent mixture is miscible, then upon evaporation of the volatile solvent, such as amyl acetate, it will be found that the nitrocellulose is retained in stable solution (or colloidal solution) in the liquid mixture of isomers. The physical properties of the product prepared in this manner are entirely different from a product prepared by simply adding nitrocellulose to the isomers. Whereas the latter absorbs large quantities of water, the product of this invention absorbs inappreciable and negligible quantities of water. The product of this invention effectively renders explosive compounds water-resistant whereas the product made by a simple mixture does not; the product of this invention enhances the disrupting, detonating and explosive characteristics of a compound, whereas the product of a simple mixture detracts from these qualities and deadens the compound.

In preparing the product of this invention, a solution is first made containing say 20 to 40 percent of nitrated cellulose (more than about 12% nitrogen content) in a suitable volatile solvent, preferably acetone. This solution is then mixed with a mixture of DNT isomers in quantity sufficient to introduce from about  $\frac{1}{2}\%$  to 10% of nitrated cellulose. The mixture is then slowly agitated and, if desired, heated to above the boiling point of the original solvent, the vapors of the solvent being carried off and separately condensed for reuse in cyclic operation of the process. In order to produce a product eminently suited for use in explosives, from about  $1\frac{1}{4}$  to  $2\frac{1}{2}$  percent of nitrogen content should be thus incorporated in the mixture of DNT isomers.

The mixture of isomers of dinitrotoluene which is capable of being successfully used in this explosive has a low crystallizing temperature. Ordinarily, it is a liquid having a specific gravity of about 1.3. Crystallization should begin to be observed at temperatures below  $60^{\circ}$  F. and preferably at temperatures of about  $52^{\circ}$  F. Mixtures having crystallization temperatures of between  $40^{\circ}$  F. and  $60^{\circ}$  F. have been successfully used. Most of the mixture should consist of the 1-2-4 and 1-2-6 isomers of dinitrotoluene with but a minor proportion of meta isomers. The mixture of isomers should be free from sulfonic acids or free acids. The mixture, furthermore, should contain not more than about 2%-3% of compounds or substances volatile at  $100^{\circ}$  C. The presence of some toluene is not objectionable, however.

A complete explosive which has been found to have exceptionally good detonation, propagation, water-resistance and plasticity, may be

made by combining the following ingredients in the proportions stated:

|                                                       | Percent                           |
|-------------------------------------------------------|-----------------------------------|
| Sodium nitrate                                        | 19-23                             |
| Potassium chlorate                                    | 38-41                             |
| Shredded wood                                         | 13-14                             |
| Liquid DNT isomers                                    | $23\frac{1}{4}$ - $27\frac{1}{2}$ |
| Nitrocellulose (more than about 12% nitrogen content) | $1\frac{1}{4}$ - $2\frac{1}{2}$   |

It is to be understood that the nitrocellulose is incorporated with the liquid DNT isomers in the manner described above before being added to a mechanical mixture of the remaining three ingredients.

The shredded wood, mentioned in the above compound, should be a shredded uncooked wood, preferably spruce or the like, capable of passing a 20 mesh sieve but retained upon a 30 mesh sieve. Obviously, some small quantity or proportion of the wood may be slightly coarser and also slightly finer in particle size, but at least 60% of the wood should be of a size between 20 and 30 mesh. A wood shredded to pass a 14 mesh sieve and be retained on a 35 mesh sieve can be used.

The explosives coming within the scope of this invention can be used for general blasting, quarrying and mining purposes, but are particularly adaptable for mining use. The fumes involved are innocuous and as a result miners can be re-entering shafts and drifts within a few minutes after detonation without experiencing undesirable physiological effects. The explosive is rather bulky, weighing about 42 pounds per cubic foot, loose weight. In stick form a 50 pound case, net weight, of 8 by  $1\frac{1}{4}$  inch sticks will contain about 145 sticks instead of the 105 sticks of similar size contained in a 50 pound case of ammonia dynamite or nitroglycerine dynamite. In explosive and breaking effect, the explosive of this invention is equivalent to the standard 50%-60% ammonia or nitroglycerine dynamite. The standard 8 inch sticks of the explosive will propagate through an air gap of at least 1 inch and as much as  $2\frac{1}{2}$  inches when a stick is cut in half, the ends longitudinally spaced and a cap inserted in one half only. No loss in sensitivity takes place upon storage of the explosive for a prolonged period of time.

The explosive composition may be subjected to the action of water for several hours without becoming saturated and without losing its explosive characteristics. No hardening or deterioration takes place even upon exposure of the sticks to extremely high temperatures ( $120$  to  $130$  degrees F., or below  $22^{\circ}$  F.) for protracted periods of time. No bleeding, separation, or hardening takes place upon exposure to sudden or radical changes of temperature.

In the event the explosive is to be used at very low temperatures, such as temperatures below  $20^{\circ}$  F., it may be desirable to incorporate from 0.5% to 2% toluene. Incorporation of this ingredient is preferably made by mixing the toluene with the isomers of dinitrotoluene. In this relation the toluene appears to exert a crystallization-retarding effect upon the isomers of dinitrotoluene which may have a tendency to crystallize out at such low temperatures, thereby causing the mass to become more firm.

The mixture of dinitrotoluene isomers referred to hereinabove appears essential for the successful preparation of the explosive and other nitrated hydrocarbons, such as nitrobenzene, can not be substituted therefor.

I claim:

1. An industrial explosive consisting essentially of about 38% to 41% of potassium chlorate, 19% to 23% of sodium nitrate, 13% to 14% of shredded wood and 23.25% to 27.5% of a liquid mixture of dinitrotoluene isomers having an initial crystallization temperature of between 25° F. and 60° F., said liquid dinitrotoluene mixture containing from about 0.5% to 2.5% of nitrated cellulose having a nitrogen content of over 12%.

2. An industrial explosive consisting essentially of about 38% to 41% of potassium chlorate, 19% to 23% of sodium nitrate, 13% to 14% of shredded wood and 23.25% to 27.5% of a liquid mixture of dinitrotoluene isomers having an initial crystallization temperature of between 25° F. and 60° F., said liquid dinitrotoluene mixture containing from about 0.5% to 2.5% of nitrated cellulose having a nitrogen content of over 12%, 15 said explosive being characterized by its ability to retain its explosive characteristics upon storage for protracted periods of time.

3. An industrial explosive consisting essentially of about 38% to 41% of potassium chlorate, 19% to 23% of sodium nitrate, 13% to 14% of shredded wood and 23.25% to 27.5% of a liquid mixture of dinitrotoluene isomers having an initial crystallization temperature of between 25° F. and 60° F., said liquid dinitrotoluene mixture containing from about 0.5% to 2.5% of nitrated cellulose of about 12% nitrogen content, said explosive being relatively plastic, capable of exploding by propagation and influence over a gap of 1 inch or more capable of resisting water and retaining its plasticity, sensitiveness and water resistance upon storage for protracted periods of time.

4. An industrial explosive consisting essentially of alkali-chlorate, a liquid mixture of dinitrotoluene isomers, alkali nitrate and shredded wood, these ingredients being in progressively

decreasing proportions in the order stated, said industrial explosive being characterized by the presence of from about 0.5% to about 2.5% of nitrated cellulose of about 12% nitrogen content in solution in said liquid mixture of dinitrotoluene isomers, said liquid mixture of dinitrotoluene isomers having an initial crystallization temperature of between 35° F. and 60° F.

5. In a method of producing industrial explosives having water resisting properties and capable of being stored for protracted periods of time without loss of sensitiveness, the steps of: dissolving nitrated cellulose containing more than about 12% nitrogen in acetone, mixing said solution with a liquid mixture of isomers of dinitrotoluene, said liquid mixture having an initial crystallization temperature of between 35° F. and 60° F., evaporating the major portion of the acetone and incorporating the solution of nitrocellulose in said liquid dinitrotoluene in a mixture of chlorate, nitrate and shredded wood to form an industrial explosive.

6. In a method of producing industrial explosives having water resisting properties and capable of being stored for protracted periods of time without loss of sensitiveness, the steps of: dissolving nitrated cellulose containing more than about 12% nitrogen in acetone, mixing said solution with a liquid mixture of isomers of dinitrotoluene, said liquid mixture having an initial crystallization temperature of between 35° F. and 60° F., evaporating the major portion of the acetone, and then incorporating from about 23.25% to 30% by weight of said solution in a mixture of potassium chlorate, sodium nitrate and shredded wood.

7. An industrial explosive of the character defined in claim 6, in which the major portion of the shredded wood passes a 20-mesh sieve and is retained on a 30-mesh sieve.

LAUD S. BYERS.